

## UNITED STATES PATENT OFFICE

2,217,544

## METHOD OF TREATING PHOTOGRAPHIC MATERIAL TO OBTAIN COLORED PICTURES

Paul Goldfinger, Brussels-Uccle, Belgium, assignor to Béla Gaspar, Brussels, Belgium

No Drawing. Application May 20, 1939, Serial No. 274,837. In Germany May 27, 1938

## 4 Claims.

(Cl. 95—6)

The present invention relates to a treatment bath for the production of dye-images from uniformly dyed photographic silver images by treating solutions that locally destroy the dye present in the layer at the areas where metallic silver is present, and in proportion to the quantity of such silver. Aqueous solutions of hydrohalic acids are already known as treatment solutions suitable for this purpose. It is moreover known that the efficacy of such baths may be intensified by the addition of various chemicals; particularly effective accelerators are for instance dimethylquinoxaline, dioxyphenazine and aminoxyphenazine. I have found that the addition of a very small quantity of hydroiodic acid or potassium iodide has the effect of accelerating the action of hydrochloric acid to such an extent, that even a very greatly diluted solution of hydrochloric acid is effective if but a very small quantity of hydroiodic acid is added to the bath. Examples of such baths are as follows, viz.:

|                            |       |     |
|----------------------------|-------|-----|
| (1) Hydrochloric acid 1.8% | litre | 1   |
| Potassium iodide           | grams | 2.2 |
| (2) Hydrochloric acid 1.8% | litre | 1   |
| Potassium iodide           | grams | 2.2 |
| 2,3-dimethyl-quinoxaline   | gram  | 1   |
| (3) Hydrochloric acid 0.6% | litre | 1   |
| Potassium iodide           | grams | 3.3 |
| 2,3-dimethyl-quinoxaline   | gram  | 0.2 |

The increase in the efficacy of the new baths is shown by the following comparative test, viz.: 0.1% of dimethyl-quinoxaline is added to a 0.5*n* hydrochloric acid. Metallic silver images dyed with Brilliantbenzoéchtgrün BL, Benzoazurine G (Schultz Farbstofftabellen, Leipzig 1931, 7th ed., vol. 1, No. 497) or with Chrysophenin G (Schultz Farbstofftabellen 1. c., No. 726) are treated with this solution and dye-images are obtained within about four minutes. If the solution contains in addition such a quantity of potassium iodide that in respect of this salt the solution is 1/75*n*, silver images dyed in the same manner are converted to dye-images much more speedily and successfully, i. e., in about one minute. A silver image dyed red with Supranolbrillantrot B (Schultz Farbstofftabellen, Leipzig 1932, 7th ed., vol. 2, page 204) when treated for six minutes in a bath without the addition of potassium iodide yields but an unsatisfactory dye-image, whereas a good dye-image is obtained within three minutes if a bath containing the potassium iodide is employed. Even the addition of a much smaller proportion of potassium iodide, say one-five-hundredth mol per litre, is still effective.

The dyes cited above are to be understood as

but examples; suitable dyes are also the other known dyes used in the art, in particular azo dyes, such as the yellow Xylenwalkgelb G (Schultz Farbstofftabellen, Leipzig 1932, 7th ed., vol. 2, page 232), the blue Diaminreinblau FF (Schultz Farbstofftabellen, Leipzig 1931, 7th ed., vol. 1 No. 510) and the red Polarbrillantrot B (Schultz Farbstofftabellen, Leipzig 1932, 7th ed., vol. 2, page 175). An addition to the bath of hydrobromic acid or bromides also is effective, but to a less degree than hydroiodic acid. On the other hand, the addition of hydroiodic acid to a hydrobromic acid bath is even more effective than to a hydrochloric acid solution, for the hydrobromic acid treating baths are in themselves more effective than hydrochloric acid solutions. However, in view of the question of greater economy, the tests as to the accelerating effect were mainly carried out in connection with hydrochloric acid baths.

In the course of these experiments, other chemicals were tested as to their accelerating effect, and it was found that not only iodides and bromides, but also sulphocyanides, such as ammonium sulphocyanides and thiocarbamide, increase the effect of a hydrochloric acid bath. These experiments were carried out with a 0.5*n* hydrochloric acid, to which was added 0.1% of dimethylquinoxaline and in addition either 0.01 mol of thiocarbamide or 0.01 mol of ammonium sulphocyanide or 0.01 mol of potassium bromide for each litre of solution. In the case of the silver image dyed with Diaminreinblau FF, the bath containing thiocarbamide had the speediest effect. When the images were dyed with Benzolichtrot (Schultz Farbstofftabellen, Leipzig 1931, 7th ed., vol. 1, No. 566) or with Brilliantbenzoéchtgrün BL, it turned out that potassium bromide and ammonium sulphocyanide had the greatest accelerating effect. On the other hand, in every experiment it was found that the effect of thiocarbamide, sulphocyanide and bromide was surpassed by the effect of the iodide. The effect of the additional component to the bath appears to be due to the fact that the substances used, and especially the hydroiodic acid, reduce the concentration of free silver ions in the aqueous solution to a greater extent than does the hydrochloric acid.

It will probably also be due to this fact that the hydroiodic acid or other substance added to the solution may be employed in such a quantity that the hydrochloric acid is present in an excess to the equivalent amount of the added substance. When using hydroiodic acid as the addition to

hydrochloric acid, useful baths were obtained when the concentration of the solution in respect of hydrochloric acid was from  $0.1n$  to normal, and in respect of hydroiodic acid from  $0.002n$  to  $0.1n$ . It follows as a matter of course that higher or lower concentrations are quite possible, and that the limits mentioned above designate only a range of concentration that is to be recommended for practical purposes.

10 What is claimed is:

1. For the production of colored photographic pictures by means of local destruction of the dye at areas where metallic silver is present in photographic layers uniformly dyed with reduc-

15 ble dyes, a treating bath comprising an acid aqueous solution of hydrochloric acid and hydroiodic acid, the concentration of chloride ions ranging from 0.1 normal to 1.0 normal, the concentration of iodide ions ranging from 0.002 normal to 0.1 normal.

20 2. For the production of colored photographic pictures by means of local destruction of the dye at areas where metallic silver is present in photographic layers uniformly dyed with reduc-  
25 ble dyes, a treating bath comprising an acid aqueous solution of hydrochloric acid and hy-

droiodic acid, the concentration of chloride ions ranging from 0.1 normal to 1.0 normal, the concentration of iodide ions ranging from 0.002 normal to 0.1 normal, the bath further comprising a small amount of dimethyl-quinoxaline.

5

3. For the production of colored photographic pictures by means of local destruction of the dye at areas where metallic silver is present in photographic layers uniformly dyed with reducible dyes, a treating bath comprising hydroiodic acid and hydrochloric acid in an at least ten-fold excess to the equivalent amount of hydroiodic acid, the concentration of the iodide ions ranging from 0.002-normal to 0.1-normal.

10

4. For the production of colored photographic pictures by means of local destruction of the dye at areas where metallic silver is present in photographic layers uniformly dyed with reducible dyes, a treating bath comprising hydroiodic acid and hydrochloric acid in an at least ten-fold excess to the equivalent amount of hydroiodic acid, the concentration of the iodide ions ranging from 0.002-normal to 0.1-normal, the bath further comprising a small amount of an organic catalyst.

15

20

25

PAUL GOLDFINGER.